

March 29, 1938.

C. B. SAWYER ET AL

**2,112,636**

## METHOD OF MAKING PIEZOELECTRIC UNITS

Filed Sept. 2, 1936



Fig. I.



FIG. 8.



FIG. 2.



63



Fig. 4



FIG. 5.



Fig. 6.



10



Fig. 7



Fig. 9.



6-14



FIG. 12



FIG. 13.

FIG. 14.

INVENTORS:  
C. B. Sawyer  
C. H. Tower and  
A. L. W. Williams  
by Ray Stahr ATTORNEY

Patented Mar. 29, 1938

2,112,636

# UNITED STATES PATENT OFFICE

2,112,636

## METHOD OF MAKING PIEZOELECTRIC UNITS

Charles B. Sawyer, Charles H. Tower, and Alfred L. W. Williams, Cleveland, Ohio, assignors to The Brush Development Company, Cleveland, Ohio, a corporation of Ohio

Application September 2, 1936, Serial No. 99,154

10 Claims. (Cl. 171—327)

This invention relates to piezo-electric crystal units and more particularly to methods of producing such units.

The object of the invention is to provide a simple and efficient method of producing a piezo-electric unit having one or more relatively thin plates or elements of Rochelle salt or similar material.

Piezo-electric units of a type employing a plate 10 of Rochelle salt or similar material cemented to a restraining body to oppose the piezo-electric deformations of the plate are now well known. U. S. Patent 1,803,274 discloses a unit of the flexing type employing a plate of crystalline material and a non-piezo-electric plate cemented together, the non-piezo-electric plate acting as a restraining body to oppose the piezo-electric deformations of the crystalline plate. U. S. Patents Reissue 20,213 and 1,803,275 disclose flexing 15 units employing two or more crystalline plates cemented together in opposition, each plate acting as a restraining body for the other plate. Sawyer and Tower in Physical Review, Vol. 35, No. 3, February 1, 1930, pages 269 to 273, have 20 shown that this restrained crystal construction reduces temperature and saturation effects.

In many applications of piezo-electric material, especially of Rochelle salt plates, it is essential that the plate be made very thin. Indeed 30 for some applications the most desirable results are secured with plates having a thickness of from .003 to .004 inch. However, prior to the present invention the difficulties of constructing such thin plates and units embodying such plates 35 were exceedingly great because of the difficulties of reducing the plates to the desired degree of thinness and the great tendency of the thin plates to fracture in applying electrodes to them and in cementing them to each other or to other 40 bodies especially where considerable pressure was necessary to drive out excess cement between the plates or to force the plates into close contact.

In order to overcome these difficulties we have 45 devised the following method. Relatively thick plates of Rochelle salt with parallel faces are first formed from slabs of such crystalline material. This can be done by sawing the slabs into the plate form and milling the sawed plates to uniform thickness such as to afford sufficient rigidity 50 and strength to withstand the stresses incident to the handling, electroding and cementing of the plates. A thickness of about  $\frac{1}{16}$  of an inch has been found satisfactory in most cases, the optimum thickness depending somewhat on the 55 other dimensions of the plate. Assuming that a

unit is to be constructed comprising a single plate of crystalline material and a non-piezo-electric restraining body as, for example, in U. S. Patent 1,803,274, an electrode is applied to one face of a relatively thick piezo-electric plate. A layer 5 of cement is then applied to this electrode surface or to the restraining body or to both and the two surfaces are brought into contact and sufficient pressure is applied to reduce the layer of cement to the desired thinness and obtain the 10 required adhesion between the plates. Due to the thickness of the crystalline plate it will withstand the forces required in this operation. The cement is then allowed to set. In case units are to be constructed employing two or more crystalline plates as shown in the aforesaid Patents Reissue 20,213 and 1,803,275, one or both of the 15 electroded surfaces of two crystalline plates are coated with cement and brought together with the application of pressure to squeeze out the excess cement, and in case the unit is to be made without inner electrodes the proper surfaces are 20 simply coated with cement and brought together under pressure and the cement allowed to set.

To reduce the crystalline plate or plates of the 25 unit to the proper thinness we provide suitable apparatus comprising a support having a flat surface to which one face of the crystal unit is attached and a cutting tool adapted to engage and remove crystalline material from the exposed face of the unit. We prefer to remove the 30 surplus crystalline material by a turning operation and to this end we provide a rotatable disk having a flat face which is very true in a plane perpendicular to the axis of rotation and having 35 a rim projecting from the surface of the disk a few thousandths of an inch. This rim preferably is a separate part movably mounted on the disk. The crystal unit is attached to the flat face of the 40 unit against the face of the disk and causing the exposed face of the unit to be subjected to a substantially greater atmospheric pressure than the other face thereof so that atmospheric pressure is utilized in holding the crystal unit on 45 the disk. This can be accomplished by providing air recesses and passages in the disk structure by means of which air may be drawn away from the under side of the unit; but we prefer to provide the necessary pressure difference by a different procedure. In such other procedure the flat surface of the disk is covered with a thin 50 layer or coating of a suitable viscous substance. A material well suited to this purpose consists of a mixture by weight of 5 parts vaseline, 2 55

parts paraffine, and 1 part rosin. We have also successfully used such materials as cup grease and cylinder oil. When the coating has been applied to the surface of the disk crystal units are 5 pressed into the coating and down to the surface of the disk, the units preferably being given a rubbing or sliding movement to secure a good contact with the disk and attain sufficient adhesion. Any number of crystal units up to the capacity of the surface of the disk may be set on, 10 in this manner. The disk is then revolved at suitable speed and a cutting tool with the surfaces whose intersection forms the cutting edge making quite a steep angle with the plane of the 15 face of the disk is preferably brought in contact with the edges of the crystal units nearest the center and gradually fed towards the periphery of the disk and parallel to the surface thereof. The tool may if desired be fed from the periphery toward the center but a sufficiently light cut 20 should be taken to prevent forcing the units in toward the center. In practice an average cutting speed of about 2000 feet per minute has been found satisfactory. The angle leading from the 25 cutting edge of the tool may be very much more acute than is the common practice in turning operations because not much effort is required to remove the somewhat friable crystalline material so that there is only a moderate amount 30 of heat to be carried away. When the edge of the tool has reached the edge of the disk a known amount of crystalline material will have been removed from the surfaces of the crystal units. This cutting process may be repeated until 35 sufficient crystalline material has been removed from the outermost surfaces of the units to bring the plates to the desired degree of thinness.

If the crystal units are of the multiple plate type they are then removed from the disk and 40 replaced thereon with the faces which have just been operated upon next to the face of the disk. The turning process is now repeated until the exposed surface is brought to the same distance from the cemented junctions as are the opposite 45 surfaces of the units. The thin cemented crystal units are now removed from the surface plate. These units with their laminated structure, though thin, are strong enough to withstand the handling incident to the removal of the grease 50 and the application of electrodes to their outer surfaces.

It is to be observed that the viscous coating employed as above described serves not merely to prevent access of air to the supported side 55 of the crystal plate or unit during the cutting operation thus utilizing the atmospheric pressure on the other face to hold the unit and disk in contact, but also, by filling in any slight depressions or irregularities in the surface of the crystal plate, to form a continuous support for the surface of said plate so as to minimize breakage of the crystalline plates during the machining operation. In addition, the viscous material of course also helps by adhesion to hold the crystal plate in position on the rotating disk.

As further illustrating and explaining the invention we have shown in the accompanying drawing several specific embodiments of our improved piezo-electric crystal units and turning apparatus for use in carrying out our improved method of producing the units.

In the drawing,

Figs. 1 and 2 are face and edge views, respectively, of a relatively thick plate of Rochelle salt 75 crystal such as is formed in the manner above

described, a portion of the plate being shown in section in Fig. 2.

Fig. 3 is an edge view of a relatively thin plate of Rochelle salt produced from the plate shown in Figs. 1 and 2 by means of our improved method, a portion of the plate being shown in section.

Fig. 4 is an edge view, partly in section, of an unfinished crystal unit consisting of two such plates as are shown in Figs. 1 and 2, with electrodes applied to their adjacent faces and with the two plates cemented together, the space between the two plates being exaggerated in order to more clearly show the electrodes.

Fig. 5 is an edge view, partly in section, of the same crystal unit after one of the plates has been turned down to the desired degree of thinness.

Fig. 6 is a similar edge view of the same unit after both plates have been turned down to the desired degree of thinness.

Fig. 7 is an edge view, partly in section, of the same crystal unit after electrodes have been applied to the outer faces of the crystal plates.

Figs. 8 and 9 are, respectively, face and edge views of a plate of Rochelle salt crystal similar 25 to that shown in Figs. 1 and 2, the plate being shown partly in section in Fig. 9.

Fig. 10 is an edge view, partly in section, of a partially completed piezo-electric unit consisting 30 of a crystal plate such as is shown in Figs. 8 and 9 cemented to the face of a metal plate.

Fig. 11 is an edge view, partly in section, of the same unit with the crystal plate turned down to the desired degree of thinness.

Fig. 12 is an edge view, partly in section, of the same unit with an electrode applied to the exposed face of the crystal plate and electric leads attached to the electrode and the metal plate, respectively.

Figs. 13 and 14, are, respectively, a front or side 40 elevation, partly in section, and a face elevation of a rotatably mounted disk of the character previously referred to adapted for use in turning down the crystal plates to the desired degree of thinness, a number of crystal units being shown 45 on the disk to better illustrate the turning operation.

Referring in detail to the structures illustrated in the drawing, and first to the crystal illustrated in Figs. 1 to 3, 1 is a relatively thick rectangular 50 plate cut from a Rochelle salt crystal or slab as previously described and 1a represents the plate after it has been turned down to the desired degree of thinness by our improved method.

Referring to the production of the piezo-electric unit shown in Fig. 7, as that production is illustrated by Figs. 4 to 7, inclusive, each of two Rochelle salt crystal plates 2, 2 of the same character as the plate 1, has an electrode 3 applied to one of its faces. The two electroded faces 60 of the two plates are then cemented together with an electrode lead 3a between them as indicated in Fig. 4. As the plates 2, 2 are relatively thick and correspondingly strong, the application of the electrodes to their surfaces and the cementing together of the two plates can readily be effected without serious danger of breakage of the plates. One of the two plates is then turned down to a desired degree of thinness, as represented by plate 2a in Fig. 5. Then the other plate 70 is similarly turned down so that both plates 2a, 2a are of the desired degree of thinness as indicated in Fig. 6. Finally, electrodes 4, 4 are applied to the outer faces of the unit, each electrode being provided with a suitable lead 4a and 75

the two leads being brought together as indicated in Fig. 7. During the reduction of thickness of the two crystal plates each is supported and strengthened by the other. It will be understood 5 that the thickness of the plates of the finished unit may be made much smaller than shown in the drawing, a total thickness for the unit of .020 inch or less being easily obtained.

In the production of the piezo-electric unit 10 shown in Fig. 12 some modification of the above described procedure is involved. Here a relatively thick rectangular plate 5 of Rochelle salt crystal, of the same character as the plates 1 and 2 above described, has one face cemented to the 15 face of a restraining member in the form of a rectangular metal plate 6 of the same size, producing an unfinished unit as shown in Fig. 10. A portion of the crystalline material of the plate 5 is then removed to reduce the thickness of said 20 plate, leaving the unit in the form shown in Fig. 11 in which the crystal plate is represented by the numeral 5a. Finally, an electrode 7 is applied to the outer face of plate 5a and a lead 7a attached to the unit. The metal plate 6 itself serves as an 25 electrode on the opposite side of plate 5a and has a lead 6a attached thereto. Alternatively, an electrode may be applied to the inner face of the thick plate 5 before the latter is cemented to the metal plate 6 and this is preferable in at least 30 some instances as giving closer contact between the electrode and the crystal plate.

Referring now to the turning apparatus shown in Figs. 13 and 14, 8 is a disk having integral or 35 rigid therewith a shaft 9 which can be rotatably mounted in any suitable bearing supports (not shown) and driven in any desired manner by power. The disk 8 is formed with a smooth face 8a constituting substantially a true plane surface at right angles to the axis of rotation of the disk. 40 A rim 10 is mounted on the periphery of the disk 8 with a loose fit. In the normal position of the rim 10 one edge of it projects beyond the surface or face 8a of the disk. The rim 10 is held in such 45 normal position by means of screws 11, 11 which extend through slots 10a in the rim. The screws are provided with knurled heads and by loosening them the rim 10 can be moved on the disk 8 so as not to extend beyond the face 8a.

At 12 is shown a turning tool adapted to cooperate with the rotatably mounted disk 8. The tool 12 can be mounted in any well known manner upon a tool support such as is employed in turning lathes and which is adapted to be adjusted manually and fed mechanically parallel to the face of 55 the disk 8.

In the use of the turning apparatus, the face 8a of the disk is covered with a coating of some suitable viscous substance, such as has been referred to. Then the disk is loaded with the work to be 60 turned down by selecting units such as those shown in Figs. 2, 4 or 10, and pressing such units firmly into the viscous coating of the face 8a of the rotatable disk. As shown in Fig. 13, the disk has been loaded with seven units 13, 13 of the 65 character illustrated in Fig. 4. The tool 12 having been set near the center of the disk and manually adjusted the right distance from the face 8a of the disk, the machine is started with the disk rotating in clock wise direction as indicated by the 70 arrow in Fig. 14 and with the feed movement of the tool toward the periphery of the disk and parallel to the face thereof. As the tool engages the crystal units the crystalline material is gradually cut away as will readily be understood. It is 75 found that the crystal units adhere strongly to

the face of the rotating disk, any movement of the work in relation to the disk being parallel to the face thereof. Under the light pressure of the tool and the centrifugal force of the rotating units there tends to be a creeping of the crystal units 5 toward the periphery of the disk but any movement of the work beyond the periphery of the disk proper is prevented by the rim 10.

When the cutting tool has progressed to the rim 10 of the rotating disk, if more material is to be removed from the same side of the crystal units the tool is reset near the center of the disk and the cutting operation repeated. In this manner the desired amount of crystalline material can be removed. When the desired amount of material has 15 been removed from one side of the unit, the securing screws 11, 11 are loosened and the rim 12 slipped back on the disk 8 so that the crystal units can be slid radially outward off the face of the disk. The adherence of the crystal units to the 20 face of the disk is so strong that it would be difficult otherwise to remove the units.

To complete these same crystal units they are removed from the disk in the manner stated and replaced with their thin crystal plates against the 25 disk so that their thicker plates are in position to be engaged by the cutting tool. The thicker plates are then turned down, in the manner described above, to the same thinness as the other plates.

We have deemed it unnecessary to illustrate 30 crystal units having more than two crystal plates and to describe the application of our process to such units and plates since it is clear and obvious that the process can advantageously be used to produce such units, the essential principle involved in all cases in which a unit is to be made comprising a thin crystalline plate cemented to another member or body, being that a relatively thick plate of the crystalline material is cemented to the other member (either another thick plate 35 of the crystalline material or a non-piezo-electric restraining member) and is then reduced to the desired thin form while the unit is supported by the other member. Thus, if four-plate units such as are described in United States Letters Patent 45 1,803,275 are to be produced, one possible procedure is to produce a two-plate unit in the manner already described and then to cement crystal plates to the faces of the two-plate unit and turn 50 them down to the desired thinness by the same sort of procedure. Such a method of producing the four-plate unit obviously embodies the above noted principle of our method. It will also be obvious that still other ways of proceeding, embodying our basic principle, can be followed to 55 produce units having more than two elements.

It should be understood that in its broader aspects our improved method is not limited to the employment of a turning operation to reduce the thickness of the crystalline plates. Obviously 60 the crystalline material can be removed by a milling operation, a shaping operation or other suitable machining operation and in any such case the support to the face of which the crystal unit is attached may be stationary and the cutters 65 moved in relation to it or the support may be moved in relation to the cutting tool. However, we consider the turning operation as described the preferable procedure because it is simple, rapid and effective and minimizes cracking and 70 breakage of the crystalline units. Since, in the turning operation, the tool has contact with a given point on the crystalline surface for a comparatively short length of time and this part of the crystalline surface has a chance to dissipate 75

whatever heat may be generated before again coming in contact with the tool and since the circulation of air caused by moving the crystal unit rather than the tool also reduces local heating 5 of the crystalline material to a minimum, cracking and breakage of the units from unequal expansion of the crystalline material are largely obviated. It should be further understood that while we have described our method as applied 10 to the production of Rochelle salt units, it is equally adapted to production of units of other mechanically similar piezo-electric material.

By the process which we have described we are able to produce on a commercial basis and with 15 but slight loss from breakage large quantities of crystal units of Rochelle salt or the like having crystalline plates as thin as two and one half to three thousandths of an inch, and are able to produce very thin single plates of crystalline material and maintain the thickness of these units and plates within very strict limits so that they may be used interchangeably in various pieces of apparatus. By means of our improved process 20 it is possible to make the individual crystal plates of multiple-plate units such as are shown in Figs. 7 and 12 thinner without undue breakage than is possible where individual plates alone are turned down to thin form. This, as has been explained, is due to the fact that in our improved 25 method of producing the multiple-plate units each plate supports and strengthens the other during the operations of cutting and application of external electrodes.

Obviously the piezo-electric units produced by 30 our method may take various forms in addition to those illustrated. For example, a unit similar to that shown in Fig. 7 may be produced without the lead 3a and with entirely separate leads attached to the external electrodes 4, 4 this being 35 a known form of units of this character. Similarly such two-plate units may be made with the complete omission of the internal electrodes 3, 3 entirely separate leads in this case also being provided for the outer electrodes 4, 4. Likewise the 40 method of producing the units can be modified in various ways, the scope of the invention being indicated by the appended claims.

What we claim is:

1. The method of making a piezo-electric unit 45 comprising one or more thin plates of frangible crystalline material which comprises forming a relatively thick plate of said material, permanently cementing one face of the plate to the surface of another body, and effecting relative movement between the resulting unit and a cutting tool to cut away crystalline material from the exposed face of the crystal plate until the latter is reduced to the desired degree of thinness.

2. A method of forming a built-up piezo-electric unit comprising two or more thin plates of frangible crystalline material which comprises cementing together face to face two relatively thick plates of the said material, supporting the resulting unit by the first of said thick plates, 50 while said unit is so supported removing crystalline material from the exposed face of the second thick plate until the latter is reduced to a desired degree of thinness, and thereafter as a final step removing crystalline material from an 55 exposed face of the first thick plate to reduce it to a desired degree of thinness while supporting the unit by a plate thereof already reduced in thickness.

3. The method of making a piezo-electric unit 60 consisting of a thin plate of frangible crystalline

material and a body of non-piezo-electric material which comprises forming a relatively thick plate of the crystalline material, permanently cementing one face of the said thick plate to the surface of the non-piezo-electric body, and effecting relative movement between the resulting unit and a cutting tool to cut away crystalline material from the exposed face of the crystal plate until the latter is reduced to the desired degree of thinness.

4. The method of making a piezo-electric unit 65 comprising one or more thin plates of frangible crystalline material which consists in forming a relatively thick plate of said material, permanently cementing one face of the plate to the surface of another body with electrode material at the junction of the said face and surface, effecting relative movement between the resulting unit and a cutting tool to cut away crystalline material from the exposed face of the crystal 70 plate until the latter is reduced to the desired degree of thinness, and thereafter applying an electrode to the exposed face of the thin crystalline plate.

5. The method of making a piezo-electric unit 75 comprising a plurality of thin plates of frangible crystalline material which comprises cementing together face to face two relatively thick plates of the said material, supporting the resulting unit by one of the plates while removing crystalline material from the exposed face of the other plate until the latter is reduced to the desired degree of thinness, and, while supporting the said unit by the thinner plate, removing crystalline material from the exposed face of the thicker plate until the latter also is reduced to the desired 80 degree of thinness.

6. The method of making a piezo-electric unit 85 comprising a plurality of thin plates of frangible crystalline material which comprises cementing together face to face two relatively thick plates of the said material, supporting the resulting unit by one of the plates while removing crystalline material from the exposed face of the other plate until the latter is reduced to the desired degree of thinness, and, while supporting the said unit by the thinner plate, removing crystalline material from the exposed face of the thicker plate until the latter also is reduced to the desired degree of thinness, and applying electrodes to the 90 exposed faces of the two-plate unit.

7. The method of making a piezo-electric unit 95 comprising a plurality of thin plates of frangible crystalline material which comprises cementing together face to face two relatively thick plates of the said material, positioning one face of the resulting crystalline unit on a support with the exposed face of the unit subjected to a greater atmospheric pressure than the other face thereof to hold the unit on the support, effecting relative motion between the support and a cutting tool to cut away the crystalline material of the exposed face of one of the crystalline plates until it is reduced to the desired degree of thinness, thereafter positioning the crystal unit on the support with a face of the unreduced thick plate exposed, and, while holding it thereon by atmospheric pressure on its exposed surface, cutting away crystalline material of the exposed face of the thicker crystalline plate until the latter 100 also is reduced to the desired degree of thinness.

8. The method of making a piezo-electric unit 105 comprising a plurality of thin plates of frangible crystalline material which comprises cementing together face to face two relatively thick plates

of the said material, pressing one face of the resulting crystalline unit against the plane face of a support after having first applied to one of said faces a coat of viscous substance, effecting a relative motion between the support and a cutting tool to cut away the crystalline material from the face of the exposed crystalline plate until it is reduced to a desired degree of thinness, thereafter positioning the unit upon the support with a face of the unreduced thick plate exposed and with a coating of viscous substance between the unit and support, and again effecting relative motion between the support and the cutting tool to cut away crystalline material of the exposed face of the thicker plate of the unit until said plate also is reduced to a desired degree of thinness.

9. The method of making a piezo-electric unit comprising a plurality of thin plates of frangible crystalline material which comprises applying an electrode to one face of each of two relatively thick plates of the said material, cementing together the two electroded faces of said plates, positioning one face of the resulting crystalline unit on a support with the exposed face of the unit subjected to a greater atmospheric pressure than the other face thereof to hold the unit on the support, effecting relative motion between the support and a cutting tool to cut away the crystalline material of the exposed face of one of the crystalline plates until it is reduced to the desired degree of thinness, thereafter positioning the

crystal unit on the support with a face of the unreduced thick plate exposed, and, while holding it thereon by atmospheric pressure on its exposed surface, cutting away crystalline material of the exposed face of the thicker crystalline plate until the latter also is reduced to the desired degree of thinness.

10. The method of making a piezo-electric unit comprising a plurality of thin plates of frangible crystalline material which comprises applying an electrode to one face of each of two relatively thick plates of the said material, cementing together the two electroded faces of said plates, pressing one face of the resulting crystalline unit against the plane face of a support after having first applied to one of said faces a coat of viscous substance, effecting a relative motion between the support and a cutting tool to cut away the crystalline material from the face of the exposed crystalline plate until it is reduced to a desired degree of thinness, positioning the unit upon the support with a face of the unreduced thick plate exposed and with a coating of viscous substance between the unit and support, and again effecting relative motion between the support and the cutting tool to cut away crystalline material of the exposed face of the thicker plate of the unit until said plate also is reduced to a desired degree of thinness.

CHARLES B. SAWYER. 30  
CHARLES H. TOWER.  
ALFRED L. W. WILLIAMS.